

Jan. 20, 1959

J. L. MORNING

2,870,006

PROCESS FOR MELTING METALS

Filed Oct. 20, 1955

2 Sheets-Sheet 1

*Fig. 1*



INVENTOR  
JOHN L. MORNING

BY *Francis J. Crowley*

ATTORNEY

Jan. 20, 1959

J. L. MORNING

2,870,006

PROCESS FOR MELTING METALS

Filed Oct. 20, 1955

2 Sheets-Sheet 2



INVENTOR  
JOHN L. MORNING

BY *Francis J. Crowley*

ATTORNEY

1

2,870,006

## PROCESS FOR MELTING METALS

John L. Morning, Wilmington, Del., assignor to E. I. du Pont de Nemours and Company, Wilmington, Del., a corporation of Delaware

Application October 20, 1955, Serial No. 541,708

4 Claims. (Cl. 75—84)

This invention relates to an improved method of melting metals which in the molten state are reactive with refractory materials used in conventional melting processes.

Many of the higher melting point metals and alloys present special problems with regard to pouring of castings and ingots. The difficulties with which this invention is concerned are encountered in the melting process. Titanium and alloys containing a major amount of titanium serve as good examples to illustrate the problems involved and the method of this invention which overcomes them. Molten titanium is reactive with atmospheric gases and with the refractory materials which are used in melting such metals as iron. For this reason, there is the problem of containing the molten metal during the melting process. One method utilizes a titanium metal crucible surrounded by an inert atmosphere. The difficulty presented by the fact that the melting point of the container is the same as that of the material being melted is overcome by externally cooling the titanium crucible while introducing radiant heat from a source above the crucible so that the maximum heat is absorbed by the surface of the molten titanium contained within the crucible. The process is initiated by dropping particles of metal into the crucible and allowing them to become molten. By proper cooling it is possible to maintain a crucible of sufficient thickness to contain the molten metal within it. The charge is gradually built up within the crucible by subsequently dropping particles of titanium into the pool of melted metal. This method is disclosed in co-pending application of C. H. Winter, Jr., Serial No. 387,011, filed October 19, 1953.

With this type of melting process, extreme care must be taken to prevent any part of the crucible from completely melting. Furthermore, it might be expected that the crucible thickness would vary during the melting operation. The portion of the crucible which is subjected to the greatest variations in thickness is at the rim where the surface of the pool contacts the walls of the crucible. This rim of contact is known as the beach line. The temperature of the crucible is greatest at the beach line because the heat is being radiated from above, thus resulting in maximum temperatures near the surface of the pool. The Winter application realizes this problem, and special cooling means are maintained about the crucible at the beach line.

This invention makes it possible to maintain a sufficient thickness of the crucible at the beach line by a process which comprises applying radiant heat from above to a pile of metal particles contained within a titanium crucible, melting a portion of said pile by said radiant heat while introducing additional metal in particle form at a rate sufficient to maintain a pile within and above the surface of the molten metal and out of contact with the heat source, said addition of metal being continued at said rate until the complete charge is introduced into the crucible, sustaining the heating until all the metal in the crucible is in the molten state and

2

finally removing the molten metal from the crucible. When the molten metal which is being treated, has a tendency to react with atmospheric gases, the above process should be carried out in a nonreacting atmosphere.

The advantages of this invention stem from the fact that the heat is absorbed by the metal particles of the pile rather than by the molten pool. This pile offers a large surface area of high emissivity value to the heat source as contrasted to the prior method of feeding particles of titanium into a molten pool. This prior method depends upon heat transfer from the liquid metal to the solid feed, and this heat must first be transferred from the radiant heat source to the low emissivity molten metal so that a considerably lower rate of energy interchange is experienced. By using this invention, it is possible to melt titanium at temperatures above 1700° C. and at the same time maintain a temperature of not more than 1300° C. at the beach line area.

Referring now to Figure 1 of the drawing, there is shown a suitable apparatus for carrying out the process of this invention. This apparatus is a tiltable furnace having an outer corrosion-resistant shell 1 of steel, or other desired metal, internally lined with a ceramic or other suitable insulating material 2 within which, as shown, the furnacing means proper is suitably disposed. This furnacing means can comprise a bottom bowl section 3, of graphite, molybdenum or other refractory material and an upper roof section 4, also preferably composed of graphite. Suitably disposed within or otherwise associated with said roof section is an electrical resistor or similar type heating element 5 having connections with a source of current (not shown) for heating and maintaining the furnace at any desired temperature above the melting point of the metal or alloy subjected to melting and purification treatment. A furnace inlet 6 is provided in the upper section 4 through which metal can be charged to the furnace. Also provided in upper section 4 is a decontamination outlet 7 through which vaporized impurities evolved in the operation can be readily withdrawn. Usually magnesium and the magnesium chloride vapors which are evolved in the melting of titanium are retained in the system to maintain an inert atmosphere. If an excess builds up it is withdrawn through outlet 7. A crucible 8, consisting of a solid layer, or skull, of titanium metal and functioning to retain the molten metal 9 within the furnace is provided within and over the interior of bowl 3. Disposed between the lowermost part of the roof section 4 and the upper limits of the bowl 3 and crucible 8 is a heat dam element 10 preferably composed of porous graphite which projects inwardly as shown for a relatively short distance over the beach line 11 to block and thereby minimize the quantity of heat reaching the exposed crucible wall above the beach line. Externally disposed about the bowl section 3 at substantially the beach line area 11 is a suitable cooling element 12, such as a coil or cooling fingers, for circulating therethrough a suitable cooling fluid such as water or other desired coolant. This cooling element provides a higher heat loss in this area 11 so that a solid layer of titanium is maintained throughout the melting operation. A pouring spout or other suitable form of outlet 13 is provided in the bottom section 3. On tilting of the furnace about a shaft, not shown in the drawing, molten metal in purified state can be withdrawn to conventional ingot-forming or other desired solidifying and recovery means.

To form a titanium metal or alloy crucible within the above described apparatus, titanium metal or alloy sponge such as is recovered from the reduction of titanium tetrachloride with magnesium, is initially fed via inlet 6 into the refractory bowl 3. Radiant heat from heater element

5 is used to melt the metal in an inert atmosphere. The pure molten titanium or alloy which results is then cooled upon the surfaces of bowl 3 by rocking the furnace while simultaneously externally cooling the bowl 3 to a temperature below the melting point of the metal. This procedure is one method of forming the crucible. Another method would be to machine the crucible from an ingot.

In the process of this invention, a further charge of metal is fed into crucible 8 for melting and purification therein at such a rate that pile 14 is kept as large as possible without coming into contact with the roof 4. The metal particles as they approach the melting point sinter and consolidate, thus allowing additional material to be added to the furnace. Sufficient feed material can be added to the furnace by this method up to the rated capacity of the furnace. Concurrently, the lower portion of the shell 1 is water or air cooled externally to withdraw heat from the environs of the vessel. This external cooling can comprise a positive step of removing the heat, or it may involve no more than allowing the heat to pass to the surrounding atmosphere. Additional cooling of the graphite bowl and crucible is effected below the dam 10 and adjacent to and above the beach line, or melt level, 11 by circulating a cooling fluid through cooling element 12. Purification is accomplished during the melting process by withdrawing vaporized impurities through furnace outlet 7. After the metal is melted, it usually is heated above its melting point to insure that the metal will remain sufficiently fluid for a short period of time after it leaves the crucible. This additional heating is known as superheating, and it facilitates the handling of the metal in the pouring operation. The purified molten metal is then removed through pouring spout 13. It may be readily seen that the apparatus could be adapted to a continuous process by using spout 13 as an overflow. The process would comprise applying radiant heat to a continuously fed pile of metal particles extending out of a pool of the molten metal, at a temperature sufficient for pouring, continually melting said pile by said radiant heat while withdrawing the molten metal at a rate which is equivalent to the rate of the melting of the pile.

Ingot-forming apparatus which may be used to receive the molten metal is disclosed in U. S. Patent 2,085,450. However, the method of ingot-molding is not considered a part of this invention, and it is apparent that the molten titanium may be handled in accordance with prior art methods after it is removed from the furnace. It must, for obvious reasons, be maintained out of contact with oxygen and nitrogen, whether inside or outside the furnace, and accordingly, it is preferred to maintain an inert atmosphere within the system, argon or helium being suitable for this purpose. A slight pressure of a few millimeters above atmospheric within the furnace is desirable to avoid inleakage of air.

Figures 2, 3 and 4 illustrate graphically the improvements over the prior art which are obtained by the process of this invention when melting pure titanium.

Figure 2 illustrates the time-temperature pattern of the upper layer of metal in the furnace. This upper layer is that portion of the metal which is exposed to the radiant heat. It will be seen from the graph that in the prior process where a pool of molten titanium is produced and solid titanium is fed into the pool, the upper surface is superheated over the melting point of titanium metal. In the improved process, where there is a pile of metal accepting the heat from the radiant source, the temperature is considerably lower, thus showing a more efficient utilization of the heat source. The area on the graph designated as superheat is that period of the process when the temperature of the metal is raised so that it will not solidify too quickly on subsequent pouring.

Figure 3 illustrates the amount of power input vs. time of heating, and it shows that under the prior method the power to the resistors of the furnace may be slightly reduced and held at a lower value after the initial pool

of titanium is obtained. This reduction prevents too great a superheating, and at the same time it compensates for the poorer heat acceptance which occurs when the pool is formed. The improved method of operation allows a greater input of power to the heated surfaces because of the higher acceptance rate of heat in the mound of solid material. The graph also shows that the total amount of energy required to melt the metal by the new improved process is less than that of the prior process because a shorter time is required as a result of a more efficient use of the energy supplied.

Figure 4 illustrates how the beach line temperature is decreased by the improved process during most of the heating cycle. By probing the beach line area with a graphite rod at various beach line temperatures and measuring the penetration of the rod it is possible to correlate, for a particular apparatus, beach line temperatures with crucible thickness. Therefore, beach line temperature is in effect a measure of the thickness of the crucible, and it will be seen from Figure 4 that under the method of this invention beach line temperatures are lower for most of the heating cycle, and therefore there is no danger of completely melting the crucible wall.

The following examples illustrate particular modes of operating the process; these examples are presented in illustration and not in limitation of the invention.

#### Example I

The method of this invention was carried out in a skull furnace as shown in Figure 1. The furnace had a maximum capacity of about 300 lbs. of molten titanium held in a crucible of solid titanium of about 4 inches in average thickness and about 2" in thickness at the beach line area. The maximum molten pool size with a safe crucible thickness was about 16" by 28" with a 4" depth. The furnace was heated to a temperature of about 2000° C., as determined by an optical pyrometer sighted on the radiant roof, using 140 kilowatts of electrical power. A residual amount of molten titanium was observed in the furnace. Initially 50 lbs. of titanium metal sponge particles were fed at a rate of about 600 lbs. per hour. Feeding was then continued at a rate of 200 lbs. of titanium per hour to maintain a mound, or cone, of solid titanium within the furnace interior, but out of contact with the heating members. As the titanium sponge sintered and consolidated, together causing a shrinkage of volume in the feed material, additional material was continuously added to the mound. The feed was stopped when a total of 200 lbs. of titanium had been added, and the material was allowed to become molten. Beach line temperatures were carefully watched during a 30 minute holding or superheating period. Optimum beach line temperature to hold a 2" sidewall at the beach line in this experiment was 1250° C. As soon as the predetermined beach line temperature had been reached a depth of pool measurement was made. A knowledge of the furnace configuration, skull thickness and depth of molten metal allowed a ready estimate of the amount of molten metal in the furnace. A 187 lb. ingot of metal was poured from this melt. The metal ingot has satisfactory physical properties for commercial use.

A control run was carried out in the same furnace utilizing the prior art method of forming a molten pool of titanium and then feeding the solid titanium to this molten pool. The electrical power input was regulated to maintain a beach line temperature of about 1300° C. An initial feed rate of 300 lbs. of titanium per hour was maintained and then a feed rate of about 50 lbs. per hour was permitted with a power input of 150 kilowatts. A 200 lb. charge of titanium was added in 190 minutes and the same superheating holding time of 30 minutes was utilized for pouring the ingot. The quality of the ingot was about the same as that obtained by the process described above. A comparison of total melting time and

electrical energy utilized illustrates the advantages of the improved process:

| Factor                                                         | Improved Method | Prior Method |
|----------------------------------------------------------------|-----------------|--------------|
| Titanium Feed Rate, lbs. per hour                              | 206             | 50           |
| Total Furnacing Time, minutes including heating up and pouring | 270             | 405          |
| Total Electrical Energy in k. w. hours                         | 630             | 1,012        |

*Example II*

A comparison of the improved method and the prior method was carried out in further runs using the procedures outlined in Example I. In these additional tests the beach line temperatures were depressed by cooling the furnace after pouring an ingot. During the holding period of 30-40 minutes, beach line temperatures of approximately 1000° C. were utilized. At this beach line temperature a thicker sidewall (up to about 4" in thickness) was obtained, and this resulted in a small (about 100 lbs.) molten metal inventory in the furnace. A comparison of the metal melting time and electrical energy utilized illustrates the advantages of the improved process:

| Factor                                                         | Improved Method | Prior Method |
|----------------------------------------------------------------|-----------------|--------------|
| Titanium Feed Rate, lbs. per hour                              | 200             | 50           |
| Total lbs. Fed                                                 | 100             | 100          |
| Total Furnacing Time, minutes including heating up and pouring | 115             | 160          |
| Total Electrical Energy in k. w. hours                         | 300             | 400          |

While Figure 1 illustrates the feeding of titanium and removal of vaporized magnesium chloride through suitable outlets in the furnace dome, feed of solid sponge can also be effected through an opening in the beach line above the melt level but below the heat dam. In this procedure, recourse can be had to a ram or other suitable device for injecting the feed. In a continuous adaptation of this invention, the pile could be maintained against the crucible wall rather than being centrally located as shown in Figure 1. By having the pile in this location it would cover a portion of the crucible wall and thereby protect it against excessive heat.

If desired, vapors of the by-product salt and residual reducing metal which are evolved from the metal being melted, can be removed from the furnace in a stream of inert gas through suitable ports in the wall of the crucible. These volatile impurities which are evaporated during the melting may be condensed and recovered in the liquid or solid state.

While titanium has been mentioned as a suitable metal for the melting and purification treatment in this process the invention is applicable to the treatment of any metal, and more particularly to high melting point refractory metals such as titanium, zirconium, hafnium, thorium, and alloys containing as a major component at least one of said metals. The term a major component means that at least 50% of the alloy is composed of one or more of the refractory metals. Typical commercial titanium alloys such as 94% Ti, 2% Fe, 2% Cr, 2% Mo; 90.9% Ti, 1.5% Fe, 1.4% Cr, 1.2% Mo, 5% Al; 90% Ti, 6% Al, 4% V; 92% Ti, 8% Mn; 92% Ti, 4% Mn, 4% Al; 92.5% Ti, 5% Al, 2.5% Sn are suitable products for the method of this invention as are experimental alloys such as 64% Ti, 36% Al. Similar alloys of the other mentioned refractory metals are also contemplated. The size of the metal particles which are introduced into the furnace may vary. An average particle size ranging from  $\frac{1}{2}$  inch to 100 mesh is suitable and may consist of sponge particles, crystals, pressed pellets, or particles of metal such as turnings, punchings or chips. The crucible used to melt the metal should be substantially non-contaminating to the desired metal product. When pure metal is

desired the crucible should be made of the same metal and of the purity of the metal desired. When alloys are melted the crucible may be of the same composition as the alloy being melted or of a composition which will not substantially change the composition desired. When different alloy compositions are treated in a series of meltings in the same furnace, the use of a residue of metal from a previous melting, a slight melting off of metal from the wall of the crucible, and variation in the feed composition are contemplated as methods to obtain desired compositions of melted products. Minor changes in the composition of the metal charge are contemplated using these methods but by scheduling the series of meltings, crucible compositions may be obtained which minimize undesirable contamination of the desired product.

Some of the metal charge may be placed in the furnace during the pre-heating period when the furnace is being brought up to the operating range. However, this procedure is optional, and addition of the metal may be delayed until melting temperatures are reached. In either case, the charge should never be added so fast that the pile of metal builds up and contacts the radiant roof since this may result in contamination of the metal. Induction means are also suitable for heating the furnace. For example, a graphite tube may be heated by induction to temperatures in excess of about 1700° C., e. g., 1700-2400° C., and in turn heat would be radiated to a crucible below. Alternating current of 9600 cycles has been successfully used in this connection. Of course, graphite resistors or an electric arc may also serve as the heating means. When using a carbon arc, one may enclose the arc within a shielding graphite tube, so that carbon contamination is avoided. The tube will act as a radiating element for heating the charged material. Heating by other means than electricity can be substituted, provided the products of combustion and other contaminating materials do not contact the titanium and provided a surface radiating in excess of about 2000° C. can be obtained.

As previously mentioned, the interior atmosphere of the furnace must be inert; i. e., it must be unreactive with the structural materials within the heated zone as well as with the metal being melted. This can be accomplished by the use of argon, helium, krypton or other inert gases. The vapors of the by-product salt and unreacted reducing metal are also useful in maintaining the non-contaminating atmosphere. These vapors, evolved during the heating operation, can be retained in the system and in many instances there will be a sufficient amount to establish the desired atmosphere. However, if there is a deficiency of these vapors for this purpose, it is convenient to supplement them with one of the above-mentioned inert gases, such as argon. The use of these by-products avoids the necessity of supplying a purchased gas which adds to the cost of the melting operation.

55 I claim:

1. In a process of melting with radiant heat from a hot surface as the sole heat source, said melting being accomplished by applying said radiant heat to a charge of metal particles situated below said surface in a crucible 60 of metal which is maintained in the solid state by external cooling, an improvement minimizing the melting of the crucible at the beach line area where the crucible contacts the surface of the pool of molten metal formed by melting comprising shading the beach line area to minimize radiant heat transfer thereto, adding the charge of metal particles at a rate sufficient to maintain a pile of metal particles large enough to absorb a major portion of the radiant heat being transmitted to both said 65 pile and said pool, thereby preventing appreciable superheat in said pool until the melting step is substantially completed, said addition of metal being continued at said rate until the complete charge is introduced into the crucible, sustaining the application of heat and superheating the molten pool in a period of time which is sub-

stantially less than the time required for melting, and then removing the molten metal from the crucible.

2. In a process of melting with radiant heat from a hot surface as the sole heat source, said melting being accomplished by applying said radiant heat to a charge of particulate metal selected from the group consisting of titanium, zirconium, hafnium, thorium, and alloys containing as a major component at least one of said metals, situated below said surface in a crucible of the same metal as that which is to be melted, maintained in the solid state by external cooling, an improvement minimizing the melting of the crucible at the beach line area where the crucible contacts the surface of the pool of molten metal formed by melting comprising shading the beach line area to minimize radiant heat transfer thereto, adding the charge of metal particles at a rate sufficient to maintain a pile of metal particles large enough to absorb a major portion of the radiant heat being transmitted to both said pile and said pool, thereby preventing appreciable superheat in said pool until the melting step is substantially completed, said addition of metal being continued at said rate until the complete charge is introduced into the crucible, sustaining the application of heat and superheating the molten pool in a period of time which is substantially less than the time required for melting, and then removing the molten metal from the crucible.

3. The process of claim 2 in which the metal is an alloy having titanium as a major component.

4. In a process of melting with radiant heat from a hot surface as the sole heat source, said melting being accomplished by applying radiant heat to a charge of titanium

particles situated below said surface in a crucible of titanium which is maintained in the solid state by external cooling, an improvement minimizing the melting of the crucible at the beach line area where the crucible contacts the surface of the pool of molten titanium formed by melting comprising shading the beach line area to minimize radiant heat transfer thereto, adding the charge of titanium particles at a rate sufficient to maintain a pile of titanium particles large enough to absorb a major portion of the radiant heat being transmitted to both said pile and said pool, thereby preventing appreciable superheat in said pool until the melting step is substantially completed, said addition of titanium being continued at said rate until the complete charge is introduced into the crucible, sustaining the application of heat and superheating the molten pool in a period of time which is substantially less than the time required for melting, and then removing the molten titanium from the crucible.

20

References Cited in the file of this patent

UNITED STATES PATENTS

|           |         |               |
|-----------|---------|---------------|
| 2,436,124 | Sklenar | Feb. 17, 1948 |
| 2,734,244 | Herres  | Feb. 14, 1956 |

25

OTHER REFERENCES

Metallurgia, June 1949, pp. 69-76.

Transactions of the Electrochemical Society, article by Kroll et al. entitled "Melting and Casting Zirconium Metal," September 1949, vol. 96, No. 3, pp. 158-169.

The Iron Age, vol. 170, No. 16, Oct. 16, 1952, pp. 105-113.

Metal Industry, Feb. 19, 1954, pp. 143-144.

30